

Nov. 28, 1939.

H. S. ORR

2,181,462

METHOD OF MULTIPLE COLD REDUCING STRIP METALS

Filed Jan. 21, 1937



Inventor:  
HOWARD S. ORR,  
by: *Usina & Lumber*,  
his Attorneys.

## UNITED STATES PATENT OFFICE

2,181,462

METHOD OF MULTIPLE COLD REDUCING  
STRIP METALS

Howard S. Orr, Gary, Ind.

Application January 21, 1937, Serial No. 121,647

2 Claims. (Cl. 80—60)

This invention relates to an improved method of reducing strip-like metals and particularly the cold reducing of strip-like metals under tension in multiple thickness in either tandem or single stand mills.

The present practice in tension strip rolling mills is to reduce the strip as a single ply or thickness within the close final thickness tolerances demanded by the trade. Thus, for example, in rolling tin plate stock the initial strip is reduced from about .065 inch down to about .010 inch thickness with a resultant thickness variation of not over plus or minus .0005 inch. In some cases this tin plate stock must be held to a gauge variation of plus or minus .00025 inch.

To obtain such a final exacting gauge tolerance, it has not heretofore been possible to roll such strip metal in single ply wider than approximately 30 inches.

20 In the reduction under tension of automobile body stock and the like, a strip of single thickness is reduced from about .100 inch to about .038 inch with a resultant thickness tolerance around plus or minus .002 inch. Strip of this final and 25 single thickness could be rolled as wide as approximately 100 inches providing the initial hot strip and sufficiently wide reducing mills are available.

An object of this invention is to provide a 30 method of rolling, as a single strip under tension, two or more superimposed thicknesses of strip metal of substantially the same analysis, thereby increasing the output of the mill in proportion to width and/or thickness without affecting operating speeds on the same reducing mill over the same material as rolled in single ply thickness.

Another object is to provide a method of rolling as a single strip, under tension, multiple thicknesses of extremely wide and thin gauge 40 metals, whereby the width of metal rolled may be increased in proportion to the number of superimposed multiple thicknesses, with a resultant single thickness variation, of any one of the superimposed strips, comparable to the same resultant thickness variation in lesser widths as rolled singly.

These and other objects will become apparent as the description proceeds, in which:

The figure illustrates a single stand reversing 50 cold reduction mill wherein hot rolled and pickled strip metals in two or more superimposed thicknesses are reduced to the desired gauge.

Hot rolled and pickled strip is preferably coiled on reels preparatory to carrying out the reduction under my present method. The reduction in

a tension mill of this strip metal necessarily includes the superimposing of two or more of these strips on one another so that the strips may either be fed singly up to the mill and superimposed immediately before being reduced in multiple, they may be superimposed on one another onto a single reel, which latter case is preferred. In either event, it is quite imperative that the different strips that are to be superimposed be of approximately the same gauge or thickness 10 and of about the same width. In the event that one strip is longer than the other, I find it expedient to secure one end of two or more strips together thus allowing the other end of the strips to possibly extend one beyond the other. Any 15 excessive length of any one strip over the others is accordingly utilized as a single ply "leader" strip of the multiple strip coil end which "leader" strip is fed into and between the reducing rolls and suitably attached to the winding or delivery 20 means.

Thus by way of example only, I may utilize a conventional four-high reversing cold reduction mill, as shown in the figure, wherein single ply hot rolled and pickled strips 2 and 3 are superimposed on one another to form a multiple strip. One end of both of the strips 2 and 3 are welded or otherwise secured together, as shown at 4, while the other end is secured at 10 to the unwinding reel 6. In this case, the excessive length 25 of the strip 2 is secured, at 5, to the winding reel 9 and acts as the "leader" as previously described and is cut off upon the completion of the reduction of the multiple strips.

The superimposed strips 2 and 3 are fed into a 30 cold reducing mill which, for example, comprises a pair of work rolls 7 driven in any suitable manner (not shown). These rolls 7 are backed up by large diametered rolls 8. The superimposed strips are fed from the unwinding reel 6 over the guide roll 12 between the reducing rolls 7 to the winding or delivery reel 9 after passing over a guide roll 12'. The multiple strip is tensioned to any desired degree between the two oppositely disposed reels 6 and 9 and the reducing mill.

More specifically and by way of example, my method of rolling as a single strip, under tension, two or more superimposed thicknesses of strip metal increases output of the same mill 50 more or less proportionate to the increased width and thickness over the same material as rolled in single ply thickness.

Thus the present method is to roll .060 inch thick hot rolled and pickled strip down to .010

inch thick in about three passes in a single stand reversing mill with such rolling producing about sixty tons of .010 inch thick strip in an eight-hour turn as per Table A.

5

Table A

Rolling 30 inch by .060 inch hot strip to .011 inch in three passes:

| Pass                   | Gauge | Length, feet | Max. speed, ft. min. | Ave. speed | Min. per pass |
|------------------------|-------|--------------|----------------------|------------|---------------|
|                        | .060  | 900          |                      |            |               |
| 15 1                   | .028  | 1,930        | 600                  | 500        | 3.86          |
| 2                      | .017  | 3,180        | 700                  | 625        | 5.09          |
| 3                      | .011  | 4,910        | 800                  | 750        | 6.55          |
| Total time for rolling |       |              |                      |            | 15.50         |

Min. per coil=15.5+2.5 min. for changing coils=18 min. Weight per coil=5,000 pounds, finishing weight. Theoretical tonnage per eight-hour turn=

$$25 \frac{8 \times 60}{18} \times \frac{5000}{2240} = 59.5 \text{ N. T.}$$

By utilizing the same mill but changing power requirements to move the strip through the same I am able to boost the output of the same mill better than 250 per cent. in the same length of time after even making due allowances for slower speeds of rolling as per Table B.

Table B

35 Rolling three-ply 60 inch by .060 inch to .011 inch in three passes:

| Pass                   | Gauge | Length, feet | Ave. speed, ft. min. | Min. per pass |
|------------------------|-------|--------------|----------------------|---------------|
| 40 1                   | .180  | 900          |                      |               |
| 2                      | .084  | 1,930        | 300                  | 6.43          |
| 3                      | .051  | 3,180        | 400                  | 7.95          |
| Total time for rolling |       |              |                      | 24.21         |

45 Total elapsed time=24.2+5.0 min. for changing coils=29.2 min. Weight per triple coil=5,000 pounds by 6=30,000 pounds, finished weight. Theoretical tonnage per eight-hour turn=

$$50 \frac{8 \times 60}{29.2} \times \frac{30,000}{2240} = 220 \text{ N. T.}$$

In Table B, it is to be noted that the increase of strip width has been doubled (i. e., from 30 to 55 60 inches). It is entirely possible to increase the width of metal being rolled in proportion to the number of superimposed thicknesses, the only factor to be considered being the ability to produce such wide widths and thicknesses of hot rolled 60 strip and mills of sufficient width to handle such multiple thicknesses.

65 Regardless of the number of superimposed thicknesses, each of the strips will be reduced proportionately to their initial thickness and the resultant gauge variations will be within narrower limits in relation to the number of strips utilized. In any event, the resultant thickness variations of any one strip will be within and much less than the variations of a single strip 70 rolled singly and of the same width.

70 It is necessary in both my method of multiple strip reduction under tension, as well as in the present practice of reducing single ply thicknesses of strip metal, that the gauge from edge-to-edge of the finished cold reduced strip be held to within

tolerances even less than that demanded for commercial tolerances to take care of any possible end-to-end variations. For this reason, it is not at present possible to cold reduce single ply strip having a finished width to thickness ratio in excess of 3000:1 and still obtain the end-to-end as well as the edge-to-edge gauge variations at present demanded. If strip cold rolled to gauge as single ply has a width to thickness ratio greater than 10 3000:1, the end-to-end gauge variations may meet the demanded gauge tolerances but it is not possible to hold the edge-to-edge gauge tolerances.

10 By my method, I am able to overcome this difficulty and cold reduce, under tension, two or more thicknesses of superimposed strip which in 15 widths and single thicknesses is in excess of 3000:1 and still obtain the end-to-end and edge-to-edge gauge variations as demanded by the trade.

20 Thus, from the foregoing description it will be readily appreciated that in single ply rolling, the narrower the width of metal, the greater the accuracy of the final gauge can be controlled (see I and III of Table C). It necessarily follows that in the reduction, under tension, of two or more thicknesses of the same width of metal the inaccuracies of gauge are equally divided between the number of strips which go to make up the multiple strip, providing that the initial gauge of all superimposed strips prior to reduction are 25 comparable (see II of Table C).

30 If the gauge variation of multiple rolling of superimposed strips is kept within the gauge tolerance produced on single ply rolling, it is possible to utilize greater widths in proportionate 35 increase to the number of superimposed strips (see IV of Table C). Thus, I can obtain the same gauge tolerance in a 60 inch wide strip as in a 30 inch wide strip if I utilize two superimposed strips or the same gauge tolerance of a single strip 40 90 inches wide as in a 30 inch wide strip if I utilize a multiple strip of three more or less equal thicknesses.

45 If I desire to increase the width in my multiple rolling without necessarily increasing it in proportion to the number of thicknesses or plies, I may improve the accuracy of the final gauge to well within the tolerances demanded and usually secured on a single ply thickness as many times 50 narrower as the plies or thicknesses which I utilize (see V of Table C), with the additional advantage of tonnage output (see Table B).

Table C

| Symbol | Width | Gauge | Ply       | Ratio as rolled width to thickness | Gauge in relation to commercial acceptable tolerances |
|--------|-------|-------|-----------|------------------------------------|-------------------------------------------------------|
| I      | 30"   | .010  | Single... | 3000:1                             | Acceptable.                                           |
| II     | 30"   | .020  | Double... | 1500:1                             | Well within.                                          |
| III    | 60"   | .010  | Single... | 6000:1                             | Well without.                                         |
| IV     | 60"   | .020  | Double... | 3000:1                             | Acceptable.                                           |
| V      | 60"   | .030  | Triple... | 2000:1                             | Within.                                               |

65 In utilizing hot rolled and pickled strip under my method, the physical dimensions of the various strips as superimposed one on another are more or less uniform.

70 However, the strips one to another, as well as within each other, are often of varying degrees of hardness due principally, either to the varying modes of preparation, analysis or of hot strip finishing and/or coiling temperatures.

70 In reducing under tension such multiple strips which may internally vary one to the other, I am

able to reduce all such multiple strips with the same degree of reduction thus producing the same proportion of initial to final gauge in each and every ply. This is made possible because in rolling under tension, the tension distributes itself among the number of plies in direct proportion to the resistance set-up to reduction of the individual strips.

By my method of reducing, under tension, strip-like metals in multiple thicknesses I am able to obtain at least one good surface on each ply which is free from such superficial surface marks as stains, grease and oil deposits, and blemishes such as scratches, carbon pits, and marks due to irregularities in the contact surfaces of the rolls. Such a surface is extremely conducive to coating as by tin, lead, zinc, chromium, and the like.

Depending on the initial surface of the contacting rolls, various degrees of surface finish are possible on the multiple thickness reduction, under tension, of strip metal. For example, two smooth contact or work rolls will produce, on low carbon strip in multiple thickness, a uniformly dull but lustrous surface on the inner surfaces of all plies with the outer roll-contacting surface being necessarily bright and smooth. It follows that with one smooth and one rough contact roll or two rough contact rolls varying resultant surfaces may be produced.

Such strip with dull inner surfaces, for example, can be annealed without the tendency to stick as is heretofore encountered and if this same annealed strip is later given a superficial surfacing as "temper" rolling it presents an excellent surface for coating as by tinning.

While I have shown and described a specific embodiment of the present invention, it will be

understood that I do not wish to be limited exactly thereto since various modifications may be made without departing from the scope of the invention as defined by the following claims.

I claim:

1. In a method of cold rolling, as a single thickness, multiple thicknesses of strip-like metals the steps which include superimposing two or more strips of substantially the same width and thickness upon each other, reducing under tension the superimposed strips between a pair of reducing rolls, the resultant width to thickness ratio being in excess of 3000:1 and having a resultant thickness gauge variation for each and every ply less than the same ply if rolled singly, the width of said strip increased in proportion to the number of superimposed thicknesses, each of which has a resultant thickness variation comparable to a like strip rolled singly and of lesser width.

2. In a method of cold rolling as a single thickness multiple thicknesses of strip-like metals the steps which include, superimposing two or more strips of substantially the same width and thickness and of varying hardness upon each other, reducing under tension the superimposed strips between a pair of reducing rolls to decrease the final thickness gauge tolerances in direct proportion to the number of plies when compared to a single ply rolled singly of the same initial metal, the width of said strip capable of being increased in proportion to the number of superimposed thicknesses, each of which has a resultant thickness variation comparable to a like strip rolled singly and of lesser width.

HOWARD S. ORR.